

United States Patent [19]  
Jenkins

US005085667A

[11] Patent Number: 5,085,667

[45] Date of Patent: Feb. 4, 1992

- [54] STAIN RESISTANCE OF NYLON CARPET: CATIONIC-DYEABLE NYLON FIBERS DYED WITH ACID DYE
- [75] Inventor: William G. Jenkins, Lexington, Va.
- [73] Assignee: Burlington Industries, Inc., Greensboro, N.C.
- [21] Appl. No.: 552,178
- [22] Filed: Jul. 12, 1990

Related U.S. Application Data

- [63] Continuation-in-part of Ser. No. 519,237, May 4, 1990, abandoned.
- [51] Int. Cl.<sup>5</sup> ..... D06P 3/00
- [52] U.S. Cl. ..... 8/539; 8/676; 8/680; 8/681; 8/685; 8/924
- [58] Field of Search ..... 8/539, 680

- [56] References Cited

U.S. PATENT DOCUMENTS

- 3,142,662 7/1964 Huffman ..... 528/313  
3,184,436 5/1965 Magat ..... 528/321  
3,454,535 7/1969 Bodesheim et al. ..... 528/321  
3,542,743 11/1970 Flamand ..... 528/335  
3,755,255 8/1973 Lodge ..... 528/172  
3,764,585 10/1973 Siclari et al. ..... 528/248  
3,853,823 12/1974 Cleary ..... 528/336  
3,865,900 2/1975 DeCaprio et al. ..... 525/182  
3,923,749 12/1975 Howell ..... 528/313  
3,931,118 1/1976 Cleary ..... 528/335

- 3,951,923 4/1976 Cleary ..... 528/324  
3,957,734 5/1976 Radimann ..... 528/321  
4,043,749 8/1977 Huffman ..... 8/531  
4,075,378 2/1978 Anton et al. ..... 428/97  
4,083,893 4/1978 Lofquist et al. ..... 525/184  
4,097,546 6/1978 Lofquist ..... 525/183  
4,166,080 8/1979 Franks et al. ..... 525/183  
4,391,968 7/1983 Merani et al. ..... 528/321  
4,579,762 4/1986 Uccl ..... 428/95  
4,780,099 10/1988 Greschler et al. ..... 8/115.6

FOREIGN PATENT DOCUMENTS

- 0373655 6/1990 European Pat. Off. .  
55-8533 3/1980 Japan .  
53-24552 7/1981 Japan .  
56-123485 9/1981 Japan .  
1150389 4/1969 United Kingdom .  
1285489 8/1972 United Kingdom .  
1478221 6/1977 United Kingdom .

Primary Examiner—A. Lionel Clingman  
Attorney, Agent, or Firm—Nixon & Vanderhye

[57] ABSTRACT

Stain-resistant nylon, especially cationic-dyeable carpet nylon, is prepared by dyeing cationic-dyeable nylon fibers with acid or premetalized dye. Lightfastness and depth of shade of an apparent value equal to acid dyeable nylons is obtained with superior stain resistance equal to commercially available solution dyed nylon carpeting.

9 Claims, No Drawings

**STAIN RESISTANCE OF NYLON CARPET:  
CATIONIC-DYEABLE NYLON FIBERS DYED  
WITH ACID DYE**

**CROSS-REFERENCE TO RELATED  
APPLICATIONS**

This application is a continuation-in-part of earlier application Ser. No. 07/519,237, filed May 4, 1990, now abandoned.

This invention relates to improving the stain resistance, lightfastness and ozone resistance of nylon, especially nylon carpet.

**BACKGROUND OF THE INVENTION**

Stain resistant nylon carpets enjoy significant market acceptance. Stain resistance is typically imparted to nylon by treating the fiber as a solid filament or in a carpet form by the application of a chemical finish as described in the following U.S. patents to Monsanto: U.S. Pat. Nos. 4,501,591; 4,592,940; and 4,839,212.

Nylon carpet fiber is generally classified as to type, depending upon its receptivity to acid dyes and basic or cationic dyes. Cationic dyeable nylons contain  $\text{SO}_3\text{H}$  groups or  $\text{COOH}$  groups within the polymer structure in an amount sufficient to render the nylon fiber dyeable with a cationic dye which groups are receptive to cationic or basic dyes. Acid dyeable nylons are essentially conventional nylons, such as polyhexamethylene adipamide and polycaprolactam. Acid dyeable nylons vary as to type and are characterized as being weakly dyed with acid dyes, average dyed with acid dyes, or deeply dyed with acid dyes.

Cationic dyeable nylons generally exhibit inherent

dyeing procedures thought to be suited to the process of this invention are:

**Pad/Steam**

5 A dye bath is prepared as follows:

|                                                                              |      |
|------------------------------------------------------------------------------|------|
| guar gum (Celcagum V-60)                                                     | 0.3  |
| antifoam (Sedgekill AO)                                                      | 0.15 |
| wetting/penetrating agent<br>(Dyebath SS-75)                                 | 0.7  |
| premetalized acid dyestuff<br>(pH adjusted to 6.0 with monosodium phosphate) | X %  |

and applied to the cationic dyeable nylon at wet pickup of 90 to 140% based on the weight of the yarn. For proper fixation, the yarn is steamed for 6 to 12 minutes then washed, extracted, treated with a fluorchemical soil repellent and dried.

**Exhaust Dyeing**

An aqueous dyebath is prepared containing the required amount of premetalized acid dyestuff, the pH adjusted to 6.0 with monosodium phosphate and, optionally, up to 0.5% Irgasol SW, a weakly cationic complexing agent which retards the strike of the acid dye by complexing with the dye and then slowly releasing the dye to the fiber as the temperature rises, is added. The dyebath temperature, initially at 80° F., is increased at a rate of 2° F. per minute to 140° F. and held there for 15 minutes, then raised again at 2° F. per minute to 208°-212° F. Cationic dyeable nylon is then exhaust dyed for 30 to 60 minutes or longer as needed to achieve the desired depth of shade.

Illustrative cationic dyeable nylons include:

| DuPont                       | Monsanto             | Allied            | BASF            |
|------------------------------|----------------------|-------------------|-----------------|
| <u>Filament</u>              |                      |                   |                 |
| "Antron" Type 924            | "Ultron" 2360-68-JEJ |                   |                 |
| "Antron" Type 494            |                      | "Anso" Type 7L422 |                 |
| "Antron" Type 754            |                      | "Anso" Type 7K53  |                 |
| "Antron" Type 854            |                      |                   |                 |
| "Antron" Type P-695          |                      |                   |                 |
| "Antron" Lumena <sup>®</sup> |                      |                   |                 |
| Type P-807A                  |                      |                   |                 |
| <u>Nylon Staple</u>          |                      |                   |                 |
| "Antron" P-676A              | "Ultron"-750-JES     | "Anso" Type 591   | "Zeftron" W1185 |
| "Antron" P-683A              |                      |                   |                 |
| "Antron" 543A                |                      |                   |                 |
| "Antron" 547A                |                      |                   |                 |

stain resistant properties, especially to acid-type stains, as compared to other nylon types used for carpet. Cationic dyeable nylons are dyeable with selected cationic dyes, but suffer from poorer lightfastness, especially in light shades, than do comparable shades dyed on acid dyeable nylon using monosulfonated or premetalized acid dyes. This has resulted in the under-utilization of cationic dyeable nylon as a carpet fiber. The fiber's inherently useful properties which otherwise make it attractive as a carpet fiber previously have not been fully realized.

This invention provides a procedure for dyeing cationic dyeable nylon with acid and premetalized acid dyes resulting in nylon carpet having improved stain resistance and fastness properties.

The preferred techniques for practicing the invention include exhaust dyeing, pad/steam dyeing, continuous carpet dyeing and the like. Illustrative examples for

55 An affinity for cationic dyes is usually imparted by the incorporation of a monomer containing sulfonic acid groups. Thus one such modification of a polyamide fiber is obtained by adding a certain amount of sulfoisophthalic acid prior to polymerization.

Premetalized and acid dyes considered suited to the process are:

| Trade Name       | Manu-fac-turer | Color Index Name | Num-ber |
|------------------|----------------|------------------|---------|
| <u>Amichrome</u> |                |                  |         |
| Black RB         | ICI            | Acid Black 63    | —       |
| Red RB           | "              | Acid Red 226     | —       |
| <u>Atalan</u>    |                |                  |         |
| Fast Orange YF   | ATL            | Acid Orange 69   | —       |
| Orange GRE       | "              | Acid Orange 62   | —       |
| Yellow GR        | "              | Acid Yellow 99   | 13900   |
| <u>Inochrome</u> |                |                  |         |
| Black BNI        | ICI            | Acid Black 52    | —       |

-continued

| Trade Name           | Manufacturer | Color Index Name | Number |
|----------------------|--------------|------------------|--------|
| <u>Intrachrome</u>   |              |                  |        |
| Black RPL            | C&K          | —                | —      |
| Black WA Ex Conc     | "            | Acid Black 52    | 15711  |
| Bordeaux RM          | "            | Acid Red 194     | —      |
| Grey RC              | "            | Acid Black 127   | —      |
| Orange G             | "            | Acid Orange 74   | —      |
| Yellow GR Conc       | "            | Acid Yellow 99   | 13900  |
| <u>Intralane</u>     |              |                  |        |
| Black BGL 150%       | "            | Acid Black 107   | —      |
| Black M-RL           | "            | Acid Black 194   | —      |
| Bordeaux M-B         | "            | Acid Violet 90   | —      |
| Brilliant Yellow 3GL | "            | Acid Yellow 127  | —      |
| Dark Blue M-BR       | "            | —                | —      |
| Red Brown RW         | "            | —                | —      |
| Gray BL 200%         | "            | Acid Black 60    | —      |
| Navy NLF             | "            | —                | —      |
| Orange RDL           | "            | Acid Orange 60   | 18732  |
| Yellow 2GL Extra     | "            | Acid Yellow 129  | —      |
| Yellow GL-S          | "            | —                | —      |
| Yellow NW            | "            | Acid Yellow 151  | 13906  |
| <u>Irgalan</u>       |              |                  |        |
| Black BGL            | Ciba-Geigy   | Acid Blk 107     | —      |
| Black GBL            | "            | —                | —      |
| Black RBL            | "            | Acid Black 132   | —      |
| Bordeaux EL          | "            | Acid Red 251     | —      |
| Bordeaux GRL 200%    | "            | Acid Red 213     | —      |
| Brown 2RL            | "            | Acid Brown 45    | —      |
| Gray BL              | "            | Acid Black 58    | —      |
| Gray BRLA            | "            | Acid Black 60    | —      |
| Olive 3BL            | "            | Acid Green 70    | —      |
| Orange 2RL           | "            | Acid Orange 60   | —      |
| Orange RL            | "            | Acid Orange 86   | —      |
| Red B 200%           | "            | Acid Red 182     | —      |
| Red 2GL              | "            | Acid Red 211     | —      |
| Yellow DRL           | "            | Acid Yellow 151  | 13906  |
| Yellow 2GL           | "            | Acid Yellow 129  | —      |
| <u>Irganol</u>       |              |                  |        |
| Brilliant Yellow     | Ciba-Geigy   | Acid Yellow 127  | —      |
| 3GLS                 |              |                  |        |
| <u>Isolan</u>        |              |                  |        |
| Black RL, Liq        | Mobay        | Acid Black 139   | —      |
| Bordeaux R 220%      | "            | Acid Red 182     | —      |
| Brown S-RL           | "            | Acid Brown 413   | —      |
| Grey KP-BL 200       | "            | —                | —      |
| Navy Blue S-RL       | "            | Acid Blue 335    | —      |
| Red S-RL             | "            | Acid Red 414     | —      |
| Yellow K-PRL 200%    | "            | Acid Yellow 137  | —      |
| Yellow NW 250%       | "            | Acid Yellow 151  | 13906  |
| Yellow S-GL          | "            | Acid Yellow 232  | —      |
| <u>Lanaperl</u>      |              |                  |        |
| Blue GN 200          | Hoechst      | Acid Blue 41     | —      |
| Blue GN              | "            | Acid Blue 40     | 62125  |
| Fast Navy Blue R 200 | "            | Acid Blue 113    | —      |
| Turquoise Blue GL    | "            | —                | —      |
| <u>Lanasyne</u>      |              |                  |        |
| Black BGL 200%       | Sandoz       | Acid Black 131   | —      |
| Black BRL 200%       | "            | Acid Black 132   | —      |
| Black S-DL, Liq      | "            | Acid Black 194   | —      |
| Black S-GL, Liq      | "            | Acid Black 222   | —      |
| Black S-RL, Liq      | "            | Acid Black 218   | —      |
| Bordeaux GRL         | "            | Acid Red 213     | —      |
| Bordeaux RL          | "            | Acid Red 217     | —      |
| Brown 2GL            | "            | Acid Brown 304   | —      |
| Carbon BL            | "            | Acid Black 170   | —      |
| Dark Brown S-BL      | "            | Acid Brown 289   | —      |
| Dark Brown S-GL      | "            | Acid Brown 298   | —      |
| Grey BL              | "            | Acid Black 58    | —      |
| Grey BLR             | "            | Acid Black 60    | 18165  |
| Navy S-BL, Liq       | "            | Acid Blue 296    | —      |
| Navy S-DNL           | "            | —                | —      |
| Olive Green S-4GL    | "            | Acid Green 106   | —      |
| Olive S-2GL          | "            | Acid Green 106   | —      |
| Orange S-RL          | "            | Acid Orange 168  | —      |
| Red 2GLN             | "            | Acid Red 404     | —      |
| Red S-G, Liq         | "            | Acid Red 399     | —      |
| Rubine S-5BL         | "            | Acid Violet 125  | —      |
| Yellow LNW           | "            | Acid Yellow 151  | 13906  |
| Yellow 2RL           | "            | Acid Orange 80   | —      |

-continued

| Trade Name                                                                                                                                     | Manufacturer | Color Index Name | Number |
|------------------------------------------------------------------------------------------------------------------------------------------------|--------------|------------------|--------|
| Yellow S-2GL, Liq                                                                                                                              | "            | Acid Yellow 235  | —      |
| <u>Levalan</u>                                                                                                                                 |              |                  |        |
| Brown I-BRL Cold                                                                                                                               | Mobay        | Acid Brown 330   | —      |
| SOL                                                                                                                                            |              |                  |        |
| Dark Brown I-TL                                                                                                                                | "            | Acid Brown 331   | —      |
| Neolan                                                                                                                                         |              |                  |        |
| 10 Black WA                                                                                                                                    | Ciba-Geigy   | Acid Black 52    | 15711  |
| Blue 2G Conc                                                                                                                                   | "            | Acid Blue 158    | 14880  |
| Bordeaux RM 133%                                                                                                                               | "            | Acid Red 194     | —      |
| Orange G                                                                                                                                       | "            | Acid Orange 74   | 18745  |
| Pink BNA 300%                                                                                                                                  | "            | Acid Red 186     | 18810  |
| Yellow GR                                                                                                                                      | "            | Acid Yellow 99   | 13900  |
| <u>Neutrichrome</u>                                                                                                                            |              |                  |        |
| 15 M Black M-R                                                                                                                                 | ICI          | Acid Black 194   | —      |
| M Bordeaux M-B                                                                                                                                 | "            | Acid Violet 90   | 18762  |
| M Navy M-BD                                                                                                                                    | "            | —                | —      |
| M Yellow M-3R                                                                                                                                  | "            | Acid Brown 384   | —      |
| <u>Neutrichrome</u>                                                                                                                            |              |                  |        |
| 20 S Black S-2B                                                                                                                                | "            | Acid Black 224   | —      |
| S Bordeaux S-BD                                                                                                                                | "            | Acid Violet 121  | —      |
| S Brown S-2R                                                                                                                                   | "            | Acid Brown 357   | —      |
| S Grey S-BG                                                                                                                                    | "            | Acid Black 188   | —      |
| S Navy S-B                                                                                                                                     | "            | Acid Blue 284    | —      |
| S Navy S-NA                                                                                                                                    | "            | —                | —      |
| 25 S Orange S-R                                                                                                                                | "            | Acid Orange 144  | —      |
| S Red S-G                                                                                                                                      | "            | Acid Red 359     | —      |
| S Yellow S-GR                                                                                                                                  | "            | Acid Yellow 121  | 18690  |
| S Yellow S-5R                                                                                                                                  | "            | Acid Orange 120  | —      |
| <u>Orcolan</u>                                                                                                                                 |              |                  |        |
| Fast Black WAN Ex                                                                                                                              | ORC          | Acid Black 52    | 15711  |
| Fast Blue GGN                                                                                                                                  | "            | Acid Blue 158    | 15050  |
| Fast Orange GEN                                                                                                                                | "            | Acid Orange 74   | 18745  |
| Fast Orange GLE-S                                                                                                                              | "            | Acid Orange 62   | —      |
| Fast Red RN                                                                                                                                    | "            | Acid Red 183     | —      |
| Fast Yellow BELN                                                                                                                               | "            | Acid Yellow 54   | 19010  |
| Fast Yellow GRN                                                                                                                                | "            | Acid Yellow 99   | 13900  |
| 30 Neutral Black BGL                                                                                                                           | "            | Acid Black 107   | —      |
| Neutral Black BR                                                                                                                               | "            | Acid Black 194   | —      |
| Neutral Black EKC                                                                                                                              | "            | Acid Black 164   | —      |
| Ex Conc                                                                                                                                        |              |                  |        |
| Neutral Black LDS                                                                                                                              | "            | —                | —      |
| Neutral Blue GL                                                                                                                                | "            | Acid Blue 127    | 61135  |
| 40 Neutral Bordeaux BSB                                                                                                                        | "            | Acid Violet 90   | 18762  |
| Neutral Brilliant                                                                                                                              | "            | Acid Yellow 127  | —      |
| Yellow 5G                                                                                                                                      |              |                  |        |
| Neutral Brown BRL                                                                                                                              | "            | —                | —      |
| Neutral Brown 2GL                                                                                                                              | "            | Acid Brown 44    | —      |
| Neutral Brown GRS                                                                                                                              | "            | Acid Brown 282   | —      |
| Neutral Brown 2RL                                                                                                                              | "            | Acid Brown 45    | —      |
| 45 Neutral Dark Blue BR                                                                                                                        | "            | Acid Blue 193    | 15707  |
| Neutral Grey B                                                                                                                                 | "            | Acid Black 60    | —      |
| Neutral Grey BLGY-N                                                                                                                            | "            | Acid Black 58    | —      |
| Neutral Orange NR                                                                                                                              | "            | Acid Orange 60   | —      |
| Neutral Orane RL                                                                                                                               | "            | Acid Orange 86   | —      |
| 250%                                                                                                                                           |              |                  |        |
| 50 Neutral Red B                                                                                                                               | "            | Acid Red 182     | —      |
| Neutral Yellow EKL                                                                                                                             | ORC          | Acid Yellow 121  | —      |
| Ex Conc                                                                                                                                        |              |                  |        |
| Neutral Yellow 2GL                                                                                                                             | "            | Acid Yellow 129  | —      |
| Ex                                                                                                                                             |              |                  |        |
| Neutral Yellow GLSN                                                                                                                            | "            | Acid Yellow 114  | —      |
| 55 Neutral Yellow WN                                                                                                                           | "            | Acid Yellow 151  | —      |
| 250%                                                                                                                                           |              |                  |        |
| The following level dyeing acid dyes are thought to work particularly in the light depths but do not build very well as strength is increased: |              |                  |        |
| <u>Nylanthrene</u>                                                                                                                             |              |                  |        |
| 60 Black GLRT                                                                                                                                  | C&K          | —                | —      |
| Black GLWC                                                                                                                                     | "            | —                | —      |
| Blue B-AR 67% Liq                                                                                                                              | "            | —                | —      |
| Blue B-AR 200%                                                                                                                                 | "            | —                | —      |
| Blue B-GA                                                                                                                                      | "            | —                | —      |
| Blue B-NB                                                                                                                                      | "            | —                | —      |
| 65 Blue GLF                                                                                                                                    | "            | —                | —      |
| Blue LGGL                                                                                                                                      | "            | —                | —      |
| Brilliant Blue 3BLF                                                                                                                            | "            | —                | —      |
| Brilliant Blue 2RFF                                                                                                                            | "            | —                | —      |
| Brilliant Yellow                                                                                                                               | "            | Acid Yellow 49   | —      |

-continued

| Trade Name             | Manufacturer | Color Index Name  | Number |
|------------------------|--------------|-------------------|--------|
| 4NGL                   |              |                   |        |
| Brilliant Yellow       | "            | —                 | —      |
| B-NGL                  |              |                   |        |
| Brilliant Yellow       | "            | Acid Yellow 219:1 | —      |
| B-4RK                  |              | —                 | —      |
| Brilliant Yellow       | "            | —                 | —      |
| CGL p.a.f.             |              |                   |        |
| Brown RSM              | "            | —                 | —      |
| Navy LFWG              | "            | —                 | —      |
| Orange B-GN            | "            | —                 | —      |
| Orane 3G               | "            | Acid Orange 156   | —      |
| Orange SLF Conc        | "            | Acid Orange 116   | —      |
| Pink BLRF (pat)        | "            | —                 | —      |
| Red B-2B               | "            | —                 | —      |
| Red B-2BSA             | "            | Acid Red 266      | —      |
| Red B-CLN Conc         | "            | —                 | —      |
| Red 2RDF               | "            | —                 | —      |
| Red 4RL (pat)          | "            | —                 | —      |
| Rubine 5BLF            | "            | Acid Red 299      | —      |
| Scarlet B-YKS          | "            | —                 | —      |
| Scarlet GYL Ex (pat)   | "            | —                 | —      |
| Scarlet YDL p.a.f.     | "            | —                 | —      |
| Yellow FLW             | "            | Acid Yellow 159   | —      |
| Yellow RAR Liq         | "            | Acid Yellow 152   | —      |
| Yellow SL 200%         | "            | Acid Yellow 198   | —      |
| Yellow SL Liq          | "            | Acid Yellow 198   | —      |
| <u>Nylomine</u>        |              |                   |        |
| Black D-2R             | ICI          | Acid Black 172    | —      |
| Blue A-G Conc Grains   | "            | Acid Blue 25      | 62055  |
| Blue A-2R              | "            | Acid Blue 62      | 62045  |
| Blue B-3G              | "            | Acid Blue 40      | 62125  |
| Blue C-B               | "            | Acid Blue 127:1   | —      |
| Blue C-2G              | "            | Acid Blue 175     | —      |
| Blue C-3R              | "            | Acid Blue 140     | —      |
| Bordeaux C-B           | "            | Acid Red 128      | 24125  |
| Bordeaux C-3B          | "            | Acid Red 119      | —      |
| Green C-G              | "            | Acid Green 27     | 61580  |
| Green C-3G             | "            | Acid Green 28     | —      |
| Navy C-2R              | "            | Acid Blue 113     | 26360  |
| Red A-B                | "            | Acid Red 396      | —      |
| Red A-2B 100%          | "            | Acid Red 266      | —      |
| Red B-3B               | "            | Acid Red 57       | —      |
| Red C-2B               | "            | Acid Red 138      | 18073  |
| Red C-BA               | "            | Acid Red 249      | 18134  |
| Red C-G                | "            | Acid Red 151      | —      |
| Violet C-B             | "            | Acid Violet 48    | —      |
| Yellow A-G             | "            | Acid Yellow 135   | —      |
| Yellow A-G 33% Pst     | "            | Acid Yellow 135   | —      |
| Yellow A-2GA 200%      | "            | Acid Yellow 49    | —      |
| Yellow A-4R 150        | "            | Acid Yellow 199   | —      |
| <u>Nylosan</u>         |              |                   |        |
| Blue 2AL/C-2AL         | Sandoz       | Acid Blue 25      | 62055  |
| Blue E/C-BGL 200%      | "            | —                 | —      |
| Blue E/C-BRL           | "            | Acid Blue 288     | —      |
| Blue E/C-GL            | "            | Acid Blue 72      | —      |
| Blue F-GBL             | "            | Acid Blue 127:1   | —      |
| Blue F-L               | "            | Acid Blue 80      | 61585  |
| Blue F-RL              | Sandoz       | Acid Blue 247     | —      |
| Blue N-BLN             | "            | —                 | —      |
| Blue N-5GL 200%        | "            | Acid Blue 280     | —      |
| Blue PRL               | "            | Acid Blue 129     | —      |
| Bordeaux E-2BL         | "            | Acid Red 301      | —      |
| Bordeaux N-BL          | "            | Acid Red 119      | —      |
| Brilliant Blue N-FL    | "            | Acid Blue 278     | —      |
| Brilliant Green F-6GL  | "            | Acid Green 28     | —      |
| Brown N-2R             | "            | Acid Orange 51    | 26550  |
| Green F-BL, 200%       | "            | Acid Green 40     | —      |
| Navy N-RBL Conc        | "            | Acid Blue 113     | 26360  |
| Orange C-GNS/E-GNS Pat | "            | Acid Orange 156   | —      |
| Orange E-2GL           | "            | Mord Orange 6     | 26520  |
| Orange N-RL            | "            | Acid Orange 127   | —      |
| Red E-BM               | "            | —                 | —      |
| Red F-5B               | "            | Acid Red 143      | —      |
| Red F-BR               | "            | Acid Red 167      | —      |
| Red F-2R/C-2R          | "            | Acid Red 151      | 26900  |
| Red F-RL               | "            | Acid Red 263      | —      |
| Red F-RS, Conc         | "            | Acid Red 114      | 23635  |

-continued

| Trade Name            | Manufacturer | Color Index Name | Number |
|-----------------------|--------------|------------------|--------|
| Red N-2RBL            | Sandoz       | Acid Red 336     | —      |
| Rubine N-5BL, 200%    | "            | Acid Red 299     | —      |
| Scarlet F-3GL         | "            | Acid Red 111     | 23266  |
| Violet F-BL           | "            | Acid Violet 48   | —      |
| Yellow N-7GL          | "            | Acid Yellow 218  | —      |
| Yellow N-3RL          | "            | Acid Orange 67   | —      |
| <u>Tectilon</u>       |              |                  |        |
| Black GD              | Ciba-Geigy   | —                | —      |
| Blue 4GN              | "            | Acid Blue 343    | —      |
| Blue GRL              | "            | Acid Blue 25     | 62055  |
| Blue 5GS              | "            | —                | —      |
| Blue 4R               | "            | Acid Blue 277    | —      |
| Floxine KL 220%       | "            | Acid Red 257     | —      |
| Orange 3G             | "            | Acid Orange 156  | —      |
| Orange 3R             | "            | —                | —      |
| Orange 4R             | "            | —                | —      |
| Red 2B                | "            | Acid Red 361     | —      |
| Red GR                | "            | Acid Red 73      | 27290  |
| Yellow 2G             | "            | Acid Yellow 169  | —      |
| Yellow 4R             | "            | Acid Yellow 219  | —      |
| <u>Telon</u>          |              |                  |        |
| Blue ANL              | Mobay        | Acid Blue 25     | 62055  |
| Blue ANL Liq 33       | "            | Acid Blue 25     | —      |
| Blue BL 125           | "            | Acid Blue 78     | 62105  |
| Blue BRL 200          | "            | Acid Blue 324    | —      |
| Blue BRL Disp 67      | "            | Acid Blue 324    | —      |
| Blue BRL Liq 67       | "            | Acid Blue 324    | —      |
| Blue CD-FG            | "            | Acid Blue 145    | 23905  |
| Blue 2GL 200          | "            | Acid Blue 40     | 62125  |
| Blue 2GL Disp 50      | "            | Acid Blue 40     | 62125  |
| Blue 4GL              | "            | —                | —      |
| Blue RRL 182          | "            | Acid Blue 62     | 62045  |
| Fast Black LD         | "            | Acid Black 172   | —      |
| Fast Black LG Liq 40  | "            | —                | —      |
| Fast Black NW         | "            | —                | —      |
| Fast Blue A-FN        | "            | Acid Blue 264    | —      |
| Fast Blue A-3GL       | "            | Acid Blue 290    | —      |
| Fast Blue A-RW        | "            | Acid Blue 205    | —      |
| Fast Blue ESN         | "            | Acid Blue 221    | —      |
| Fast Blue 5G          | "            | Acid Blue 232    | —      |
| Fast Blue GL 200      | "            | Acid Blue 102    | 50320  |
| Fast Blue GGN         | "            | Acid Blue 127:1  | —      |
| Fast Blue RLW         | "            | Acid Blue 204    | —      |
| Fast Green BW         | "            | Acid Green 84    | —      |
| Fast Navy Blue R 182  | "            | Acid Blue 113    | 26360  |
| Fast Navy Blue RF     | "            | Acid Blue 113    | 26360  |
| Fast Orange A-RTL 200 | "            | Acid Orange 116  | —      |
| Fast Red A-FG         | "            | Acid Red 360     | —      |
| Fast Red BRL 200      | "            | Acid Red 260     | —      |
| Fast Red 3BW          | "            | Acid Red 274     | —      |
| Fast Red ER           | "            | Acid Red 158     | 20530  |
| Fast Red GN           | Mobay        | Acid Red 111     | 23266  |
| Fast Rubine A5BL 167  | "            | —                | —      |
| Fast Rubine A-5BLW    | "            | Acid Red 299     | —      |
| Fast Violet A-BB      | "            | Acid Violet 103  | —      |
| Fast Yellow A-3GL     | "            | Acid Yellow 216  | —      |
| Fast Yellow A-3RL     | "            | —                | —      |
| Fast Yellow 4GL 175   | "            | Acid Yellow 79   | —      |
| Red 2BL 200           | "            | Acid Red 266     | —      |
| Red 2BL Liq 33        | "            | Acid Red 266     | —      |
| Red 2BL Disp 67       | "            | Acid Red 266     | —      |
| Red BR-CL Disp 83     | "            | —                | —      |
| Red BR-CL 250         | "            | —                | —      |
| Red CD-R              | "            | Acid Red 395     | —      |
| Red FL 200            | "            | Acid Red 337     | —      |
| Red FL Liq 33         | "            | Acid Red 337     | —      |
| Red FL Disp 67        | "            | Acid Red 337     | —      |
| Yellow FGL 200        | "            | Acid Yellow 49   | —      |
| Yellow FGL Liq 66     | "            | Acid Yellow 49   | —      |
| Yellow K-RNL 200      | "            | Acid Yellow 230  | —      |
| Yellow Brown 3GL      | "            | Acid Brown 248   | —      |

Page numbers reference AATCC® Buyer's Guideline for the Textile Wet Processing Industry

\*American Association of Textile Chemists and Colorists

The tests employed in the examples that follow are identified by their AATCC or other monograph and are briefly described as follows:

**A-2 Proposed AATCC Stain Test**

A solution of eight milligrams FD&C Red Dye No. 40 per one liter solution of distilled water is prepared with pH of the solution adjusted to 5.5 with citric acid. The temperature of this solution is maintained at 75° F.  $\pm 5^\circ$  F.

The carpet sample to be tested is placed on a flat surface, and an approximately two inch diameter cylinder (open on both ends) is placed onto the surface of the carpet. Twenty ml. of the above test solution is poured into this cylinder and allowed to absorb into the carpet, after which the cylinder is removed. The carpet is allowed to stand with the stain on it undisturbed for 24 hours. After 24 hours, the carpet is thoroughly flush rinsed under cold or cool tap water, then extracted and either dried in an oven or air dried.

The degree of staining is judged by comparing the amount of discoloration produced in the spotted area as compared to the surrounding area. The Modified Allied Stain Resistance Scale, a 10 point transparency scale, is used to provide a numerical rating. For the purpose of these studies, more interest was given to the relative staining differences between carpet samples.

**B-1—DuPont Blue Dye 1 "Stainmaster" Test**

A solution is prepared the same as the above test except eight milligrams of FD&C Blue Dye 1 is used; the test is carried out in the identical manner as the AATCC stain test just described.

**A-40—DuPont Red Dye 40 "Stainmaster" Test**

A solution of 45 grams of cherry flavored "Kool-Aid" (sweetened) in 500 ml of distilled water is prepared. The solution is maintained at 75° F.  $\pm$ . Spotting, washing, etc., is conducted the same as that described above.

**24 Hour Stain Tests Using Household Foods and Stain-Producing Products**

Twenty ml of each of the ingredients listed in the relevant example were placed on each of the three test carpet samples, allowed to stand undisturbed for 24 hours, then flush rinsed under cool tap water, extracted and dried. Any solid matter was first scraped from the surface of the carpet before rinsing. The degree of staining was judged (after drying) visually between carpet samples with no scale being available to provide numerical ratings.

The invention is further explained with reference to the following illustrative examples. All parts and percentages are by weight unless otherwise indicated.

**EXAMPLE 1**

A sample carpet was made using type 854 Antron dyed in two shades, air entangled into a 4-ply yarn, then

tangled into a level loop carpet swatch. The following dyebaths were used:

|    |                             | Beige  | Gray   |
|----|-----------------------------|--------|--------|
| 5  | Irgalan Yellow 3RL<br>200%  | .072%  | .0247% |
|    | Irgalan Bordeaux EL<br>200% | .0211% | .0045% |
|    | Irgalan Black GBL<br>200%   | .05%   | .0448% |
| 10 |                             |        |        |

Percentages (%) are based upon weight of dye to weight of fiber. Each dyebath was adjusted to pH 6 with 0.2% monosodium phosphate (MSP).

15 For performance comparisons, two previously dyed yarns 856/857 Antron (acid dyeable) of the same shade were each tufted into carpet swatches. As a control a third pair of carpet swatches was prepared from DuPont's solution dyed Antron Lumena, two ends each of 20 light grey and smoke beige.

The three sets of samples were subjected to each of tests 1, 2 and 3 identified above. The two acid dyeable Antron samples performed poorly for stain resistance, whereas the cationic-dyeable Antron 854 dyed with premetalized acid dyes according to the present invention and Antron Lumena performed very well for stain resistance in all three tests with no residual stain after washing with cold clear water and extracting.

**EXAMPLE 2**

Cationic dyeable Antron 854 stock was dyed with the following premetalized acid dyes at concentrations of 0.05, 0.1, 0.25 and 1.0%.

|    |                            |      |
|----|----------------------------|------|
|    | Bordeaux EL                | 200% |
|    | Irgalan Yellow 3RL-KWL     | 250% |
|    | Irgalan Red Brown RL       | 200% |
|    | Irgalan Blue 3GL           | 200% |
|    | Irgalan Black RBL          | 200% |
| 40 | Irganol Brilliant Blue 7GS | 200% |

at pH 6.0 adjusted with MSP. No other additives were used in the aqueous dyebath.

45 To determine the ability to build the depth of shade, a similar dyeing was made on 855 light acid dyeable Antron. The 855 yarn was only appreciably darker at the 1.0% level, indicating the ability to dye light to medium shades on 854 Antron cationic dyeable nylon with premetalized acid dyes.

**EXAMPLE 3**

Lightfastness and ozone resistance were assessed to twelve representative shades of premetalized acid dyes on cationic dyeable Antron type 854 nylon.

55 The dye constituents used to prepare the shades are as follows:

|                           | Lt Gold | Beige | Green | Blue  | Rose Beige | Dusty Rose | Rust | Burgundy | Black | Med Gray | Green Gray | Lt Blue |
|---------------------------|---------|-------|-------|-------|------------|------------|------|----------|-------|----------|------------|---------|
| Irgalan Yellow 3RL 200%   | .16%    | .12%  | .17%  | .012% | .148%      | .0115%     |      |          |       | .02%     | .074%      | .022%   |
| (Acid Orange 162)         |         |       |       |       |            |            |      |          |       |          |            |         |
| Irgalan Red Brown RL 200% | .029%   | .029% |       |       |            | .288%      | 1.0% |          |       |          | .018%      |         |
| (Acid Brown 226)          |         |       |       |       |            |            |      |          |       |          |            |         |
| Irgalan Bordeaux          |         |       |       |       | .08%       |            |      | 1.0%     |       |          |            | .007%   |

-continued

|                   | Lt Gold | Beige | Green | Blue | Rose Beige | Dusty Rose | Rust | Burgundy | Black | Med Gray | Green Gray | Lt Blue |
|-------------------|---------|-------|-------|------|------------|------------|------|----------|-------|----------|------------|---------|
| EL 200%           |         |       |       |      |            |            |      |          |       |          |            |         |
| (Acid Red 251)    |         |       |       |      |            |            |      |          |       |          |            |         |
| Irgalan Blue      | .016%   | .02%  |       |      | .288%      | .064%      |      |          |       |          | .16%       | .076%   |
| 3GL 200%          |         |       |       |      |            |            |      |          |       |          |            |         |
| (Acid Blue 171)   |         |       |       |      |            |            |      |          |       |          |            |         |
| Irganol Brilliant |         |       |       |      |            |            |      |          |       |          |            |         |
| Blue 7GS 200%     |         |       |       |      |            |            |      |          |       |          |            |         |
| (Acid Blue 239)   |         |       |       |      |            |            |      |          |       |          |            |         |
| Irgalan Black     |         |       |       |      |            |            |      |          |       |          |            |         |
| RBL 200%          |         |       |       |      |            |            |      |          |       |          |            |         |
| (Acid Black 132)  |         |       |       |      |            |            |      |          |       |          |            |         |

% dyestuff based upon the weight of the fiber

2.0% Monosodium Phosphate

pH 6.0

| Shade       | Lightfastness* |         | AATCC-Ozone<br>5 cycle |
|-------------|----------------|---------|------------------------|
|             | 120 hrs        | 200 hrs |                        |
| light gold  | 4/5            | 4       | 3                      |
| beige       | 4/5            | 4       | 2                      |
| green       | 4/5            | 3       | 3                      |
| blue        | 4/5            | 4       | 3                      |
| rose beige  | 4/5            | 4/5     | 3                      |
| dusty rose  | 5              | 4       | 2                      |
| rust        | 5              | 5       | 4                      |
| burgundy    | 5              | 4/5     | 2                      |
| black       | 4/5            | 4/5     | 4                      |
| medium gray | 5              | 4/5     | 3                      |
| green gray  | 4/5            | 4       | 3                      |
| light blue  | 4/5            | 4       | 3                      |

\*AATCC 16E

The level of lightfastness achieved performs very well under the most severe exposure conditions such as those found in direct sunlight or behind glass. In contrast, the cationic dyes began to perform poorly after only 40 hours. A grade of 3 or better after 5 cycles of ozone is accepted by the industry in tropical climates in un-air-conditioned installations.

## EXAMPLE 4

Traffic performance was evaluated using a commercial carpet construction in a two-tone gray color. Three fibers were selected:

| Name          | Type             |
|---------------|------------------|
| Antron T-854  | cationic dyeable |
| Antron Lumena | solution dyed    |
| Antrol T-857  | acid dyable      |

The cationic dyeable nylon was dyed with the premetallized dye:

|                                 |       |
|---------------------------------|-------|
| <u>Red Grey</u>                 |       |
| Irgalan Yellow 3RL-KWL 250%     | .054% |
| Irgalan Black RBL 200%          | .204% |
| <u>Green Grey</u>               |       |
| Irgalan Yellow 3RL-KWL 250%     | .083% |
| Irgalan Bordeaux EL 200%        | .022% |
| Irgalan Brilliant Blue 7GS 200% | .08%  |

Both dyeings were exhaust dyed with 0.25% Irgasol SW and 2.0% MSP to adjust the pH to 6.0. The other two carpets were used as comparisons as conventionally dyed contract carpets. All three carpets were subjected to spotting with staining agents including coffee, cherry Kool-Aid, organic-bond iodine and laundry

bleach. Each agent was applied, allowed to remain on 20 the carpet overnight, then cleaned with a water flush.

The carpet of this invention performed in an equal manner to the solution dyed carpet in all areas except resistance to household bleach where the solution dyed carpet was found to be resistant to bleach discoloration 25 whereas the carpet of this invention was not resistant. Conventionally dyed Antron type 856/857 stained heavily.

## EXAMPLE 5

30 Cationic dyeable yarn (Antron type 854) knit into a tube was continuously dyed in a laboratory Ilma pad/-steam unit with 100% wet pickup with the indicated premetallized dyes depending upon the shade desired, then steamed for approximately 8 minutes to provide the desired base shade. The base shade-dyed tube was then overprinted using a silk screen process:

Pad baths for the background shade were:

|            |                     |        |
|------------|---------------------|--------|
| Gray       | Irgalan Bordeaux EL | .015%  |
|            | Irgalan Yellow 3RL  | .015%  |
|            | Irgalan Blue 3RL    | .1487% |
| Light Gold | Irgalan Yellow 3RL  | .05%   |
|            | Celcagum V-60       | .30%   |
|            | Dyebath SS-75       | .7%    |

45 Each pad bath also included Celcagum V-60 (0.3%) and Dyebath SS-75 (0.7%) and was adjusted to pH 6 with MSP.

50 Print pastes in 4 shades were prepared from a base of thickener (Lyngum CP-3) 2.35%, penetrant (Tergitol) 1%, an antifoaming agent (Antifoam CK-2) 0.15% and adjusted to pH 6.0 with MSP. Dyes used for the 4 shades were:

|                                 |             |                                  |
|---------------------------------|-------------|----------------------------------|
| <u>Red Grey</u>                 | dark gold   | Irgalan Yellow 3RL 1%            |
| Irgalan Yellow 3RL-KWL 250%     | bright blue | Irgalan Brilliant Blue 7GS 0.25% |
| Irgalan Black RBL 200%          | burgundy    | Irgalan Bordeaux EL 200% 1%      |
| <u>Green Grey</u>               | green       | Irgalan Brilliant Blue 7GS 0.25% |
| Irgalan Yellow 3RL-KWL 250%     |             | Irgalan Yellow 3RL 0.25%         |
| Irgalan Bordeaux EL 200%        |             |                                  |
| Irgalan Brilliant Blue 7GS 200% |             |                                  |

60 The printed samples were fixed with steam, washed and dried. The print design was satisfactorily fixed to the nylon tube with good crockfastness. This dyed and space printed product offers a styling versatility advantage over solution dyed nylon, in which pigment is extruded with the polymer, by allowing multiple colors on one yarn while maintaining the antistaining advantage inherent in cationically dyed nylon yarns.

Additionally a skein of "Antron Lumena" P-807A solution pigmented yarn (colored pigment is incorporated into the polymer prior to extrusion into filament form) which also exhibits cationic dyeable properties, was printed with the same dark gold, bright blue and burgundy formulation above. This was followed by fifteen minutes atmospheric steaming at 210° F., washing and drying. The resulting overprint with the pre-metallized acid dye was judged to have acceptable crock fastness and performance as a product styling tool.

In the foregoing description, the materials identified for convenience by tradename or trademark are more specifically described in the literature and materials available to the trade as follows:

| Dyestuffs                                                     | Color Index Name |
|---------------------------------------------------------------|------------------|
| "Irgalan" Yellow 3RL 200%                                     | Acid Orange 162  |
| "Irgalan" Yellow 3RL KWL 200%<br>(cold water soluble version) | Acid Orange 162  |
| "Irgalan" Red Brown RL 200%                                   | Acid Brown 226   |
| "Irgalan" Bordeaux EL 200%                                    | Acid Red 251     |
| "Irgalan" Blue 3GL 200%                                       | Acid Blue 171    |
| "Irgalan" Black RBL 200%                                      | Acid Black 132   |
| "Irgalan" Black BGL 200%                                      | Acid Black 107   |
| "Irganol" Brilliant Blue 7GS 200%                             | Acid Blue 239    |

### Chemicals

"Irgasol" SW (Ciba Geigy Corp)—Alkyl Amino Polyglycol Ether—A non-ionic aliphatic, nitrogenous compound which complexes with the anionic dye forming addition compounds which break down as temperature rises allowing controlled exhaustion of the dye-stuff.

"Progacyl" V-60-VDMIL (Rhône-Poulenc) (formerly Celcagum V-60, Lydal Chemical)—Non-ionic Guar Gum—a derivatized, low residue, acid hydrating, non-dusty guar gum designed specifically for the carpet and textile industries.

"Progacyl" CP-3 (Rhône-Poulenc) (formerly CP3, Lyngum, Lyndal Chemical)—Anionic Guar Gum—An anionic acid hydrating, derivatized guar gum thickener.

"Sedgemul" SS-75 (Sedgefield Specialties) (formerly Dyebath SS-75, BI Chem)—An aqueous mixture of sulfated ether and alcohols—A concentrated anionic wetting agent exhibiting exceptionally rapid wetting properties at temperatures usually employed in textile processing.

"Sedgekil" CK-2 (Sedgefield Specialties) (formerly Antifoam CK-2, BI Chem)—An aqueous mixture of organosilicone, sulfactants and acrylic polymer.

"Tergitol" Non-ionic 15-S-3 (Union Carbide Corp)—A linear alcohol polyethylene glycol ether.

What is claimed is:

1. A process of dyeing cationic-dyeable nylon fibers comprising dyeing said fibers with an acid dye or a premetallized acid dye at a pH of from about 4.0 to 6.5 and fixing the dye to the fibers.

2. (twice amended) A process of preparing a stain-resistant, light fast nylon carpet comprising dyeing cationic-dyeable nylon fibers with an acid dye or a premetallized acid dye at a pH of from about 4.0 to 6.5 to impart the requisite depth of shade to the nylon fibers and heating the dye-laden fibers to fix the dye into the fibers.

3. The process of claim 1 or 2, in which the nylon fibers contain  $\text{SO}_3\text{H}$  and/or  $\text{COOH}$  groups receptive to cationic or basic dyes in an amount sufficient to render the cationic fiber dyeable with a cationic or basic dye.

4. The process of claim 1 or 2, in which the nylon fibers are dyed at a pH of from about 4.0 to 6.5.

5. The process of claim 1 or 2, in which, subsequent to dye fixation, a fluorocarbon soil repellent is applied to the fibers.

6. The process of claim 1 or 2, in which a premetallized acid dye is used.

7. Nylon carpet having improved stain resistance composed of cationic-dyeable nylon fibers dyed at a pH of from about 4.0 to 6.5 with an acid or premetallized acid dye having substantially the same fastness to light as acid dyeable nylon dyed to the corresponding shade.

8. A nylon carpet composed of cationic-dyeable nylon and dyed at a pH of from about 4.0 to 6.5 to a predetermined depth of shade with an acid dye or a premetallized acid dye, the carpet being resistant to acid type stains and exhibiting improved fastness to light as compared to cationic dyeable nylon dyed to a similar depth of shade with a cationic dye.

9. The process of claims 1 or 2, in which the nylon fibers are overprinted with acid dyes or premetallized dyes to give multiple color effects on the same strand of yarn.

\* \* \* \* \*

UNITED STATES PATENT AND TRADEMARK OFFICE  
CERTIFICATE OF CORRECTION

PATENT NO. : 5,085,667

1 of 3

DATED : February 4, 1992

INVENTOR(S) : Jenkins

It is certified that error appears in the above-identified patent and that said Letters Patent is hereby corrected as shown below: On the Title page

Add under "References Cited" the following"

|             |         |       |
|-------------|---------|-------|
| --64-221574 | 9/1989  | Japan |
| 64-260061   | 10/1989 | Japan |
| 64-223908   | 9/1989  | Japan |

Column 1, line 28, "dyeably" should be --dyeable--.

Column 2, line 16, after "minutes" insert --and--.

Column 2, line 17, "fluorchemical" should be --fluorochemical--.

Column 2, line 22, after "pH" insert --is--.

Column 2, line 24, after "SW" delete the "," comma and insert --is added. (This is --.

Column 2, line 27, delete "ing" and insert --es--.

Column 2, lines 27 and 28, delete ", is added" and insert --)--.

Column 5, line 13, "Orane" should be --Orange--.

Column 6, delete lines 64-66 (the last three lines).

Column 7, line 2, after "monograph" insert --designations--.

Column 7, line 5, before "A-2" insert --Test 1:--.

Column 7, line 29, before "B-1" insert --Test 2:--.

UNITED STATES PATENT AND TRADEMARK OFFICE  
CERTIFICATE OF CORRECTION

PATENT NO. : 5,085,667

2 of 3

DATED : February 4, 1992

INVENTOR(S) : JENKINS

It is certified that error appears in the above-identified patent and that said Letters Patent is hereby corrected as shown below:

Column 7, line 34, before "A-40" insert --Test 3:--.

Column 7, line 38 after "75°F.+" insert --5°F.--,

Column 7, line 42, before "24" insert --Test Procedure:--.

Column 7, line 45, delete "relevant example" and insert --three tests above--.

Column 7, line 45, delete "the".

Column 7, line 57, after "854" insert --cationic dyeable--.

Column 8, line 1, delete "tangled" and insert --tufted--.

Column 8, line 16, before "856/857" insert --of type--.

Column 8, line 22, delete "tests 1, 2 and 3" and insert --Tests 1, 2 and 3 according to the Test Procedure--.

Column 8, line 36, before "Bordeaux" insert --Irgalan--.

Column 8, lines 45 and 46, before each occurrence of "855" insert --type--.

Column 8, line 48, before "854" insert --type--.

UNITED STATES PATENT AND TRADEMARK OFFICE  
CERTIFICATE OF CORRECTION

PATENT NO. : 5,085,667

3 of 3

DATED : February 4, 1992

INVENTOR(S) : JENKINS

It is certified that error appears in the above-identified patent and that said Letters Patent is hereby corrected as shown below:

Column 9, line 27, delete "burgandy" and insert --burgundy--.

Column 9, line 49, delete "Antrol" and insert --Antron--.

Column 9, line 49, delete "dyable" and insert --dyeable--.

Column 9, line 52, before "premetallized" insert --following--.

Column 9, line 53, delete "dye" and insert --dyes--.

Column 9, line 68, delete "organic-bond" and insert --organic bound--.

Column 12, line 4, delete the dash "--" at the end of said line.

Column 12, line 11, delete "twice amended".

Column 12, line 16, delete "the requisite" and insert --a predetermined--.

Column 12, line 23, delete "6.5" and insert --6.0--.

Signed and Sealed this

Twenty-third Day of March, 1993

*Attest:*

STEPHEN G. KUNIN

*Attesting Officer*

*Acting Commissioner of Patents and Trademarks*

UNITED STATES PATENT AND TRADEMARK OFFICE

**CERTIFICATE OF CORRECTION**

PATENT NO. : **5,085,667**  
DATED : **February 4, 1992**  
INVENTOR(S) : **JENKINS**

It is certified that error appears in the above-identified patent and that said letters patent is hereby corrected as shown below:

Column 10, line 41, change "Irgalan Blue 3RL" to read --Irgalan Blue 3GL--.

Column 10, lines 56 and 58, change "Irgalan Brilliant Blue 7GS" to read --Irganol Brilliant Blue 7GS--.

Signed and Sealed this

Eleventh Day of November, 1997

Attest:



BRUCE LEHMAN

*Attesting Officer*

*Commissioner of Patents and Trademarks*